

## UNITED STATES PATENT OFFICE

2,335,506

## STEEL HEAT TREATMENT

Raymond A. Grange, Jersey City, N. J., assignor  
to United States Steel Corporation of Delaware,  
a corporation of Delaware

No Drawing. Application December 5, 1942,  
Serial No. 467,987

3 Claims. (Cl. 148—21.5)

This invention is concerned with decreasing harmful effects resulting when steel, of any type, contains flattened, non-metallic inclusions that are plastic at the hot-working temperature of the steel. The flattening of such inclusions results from the flattening of the steel by hot-working, the inclusions then being plastic so that they, along with the steel, become flattened, the inclusions assuming the form of plate-like bodies, or laminations, which are harmful to the steel to the extent that they adversely affect its properties. For example, such inclusions decrease the transverse ductility of hot-rolled steel plate and sheet. Obviously only the non-carbonaceous inclusions are of this character, since the carbides are not plastic at steel hot-working temperatures and, therefore, are not worked into plate-like bodies, or laminations, during hot working involving flattening of the steel.

According to the invention, steel containing such flattened, non-metallic inclusions, is heated to temperatures high enough to render these inclusions mobile, and held, at such temperatures, until the inclusions convert to discontinuous, spheroidal form. In other words, at adequately high temperatures, the inclusions coalesce into areas of discontinuous spheroids if given adequate time. The exact time and temperature required can be ascertained by heating the steel to different temperatures for different times, metallographic examinations serving to show when the temperature and time are adequate to produce the desired effect. When the inclusions assume the form of discontinuous spheroids, they do not affect the properties of steel so adversely as they do when in their flattened form.

As a specific example of the invention, S. A. E. X-4130 sheet steel, which had been worked, to a .105" thickness, so as to include sufficient hot-rolling to produce the relatively thin, flattened plates of non-metallic inclusions, prevalent in this particular steel, was heat treated in accordance with this invention, by being soaked at temperatures within the range of from about 1900° to 2300° F. for about 20 hours, while sealed in an air-tight enclosure to protect it from oxidation and decarburization, subsequent metallographic examination showing that the specified inclusions had been largely converted into discontinuous spheroids. Comparative bend tests of this steel, before and after this heat treatment, showed material improvement in its transverse ductility.

The described treatment results in a new product, namely, hot-worked, elongated steel, of any type, containing non-metallic inclusions that are plastic at the steel's hot-working temperature and which are in discontinuous, spheroidal form, as contrasted to the continuous, flattened plates of such inclusions, common to the prior art steels.

During the heat treatment, it is usually desirable to protect the steel against oxidation and, in some instances, decarburization. It is to be understood that the described heat treatment should usually be applied after all hot-working has been finished, because further hot-working might again flatten the inclusions. At the same time, the treatment may be applied just prior to the last stages of hot-rolling, if the latter does not flatten the steel too much. As previously mentioned, the invention is applicable to any type of steel containing inclusions that are plastic at the steel's hot-working temperatures, and which are flattened by hot-working of the steel so as to adversely affect the steel's properties. It is also applicable to products whose nature of hot-working results in elongated, continuous stringers of such inclusions, such as are produced in hot-rolled round shapes, if it is considered, for any reason, that such stringers are more harmful than discontinuous strings of spheroids.

I claim:

1. A method of treating steel containing elongated non-metallic, non-carbonaceous inclusions that are plastic at the hot-working temperature of the steel, comprising heating the steel to temperatures high enough to render such inclusions mobile and holding at said temperatures until said inclusions convert to discontinuous spheroidal form.

2. A method of treating steel containing elongated non-metallic, non-carbonaceous inclusions that are plastic at the hot-working temperature of the steel, comprising heating the steel to temperatures of from about 1900° to 2300° F. for a period sufficient to effect an appreciable degree of coalescence of the inclusions.

3. Hot-worked, elongated steel containing non-metallic, non-carbonaceous inclusions that are plastic at the steel's hot-working temperature and which are in discontinuous spheroidal form.

RAYMOND A. GRANGE.